

(No Model.)

J. L. REED.

ASBESTUS FACED FELT.

No. 387,368.

Patented Aug. 7, 1888.

FIG. 1.



FIG. 2.



FIG. 3.



Witnesses:

John Buckler,  
W<sup>m</sup> H. Wrightman

Inventor:

James L. Reed,  
By A. M. Pierce.  
Attorney.

# UNITED STATES PATENT OFFICE.

JAMES L. REED, OF BROOKLYN, ASSIGNOR OF FIVE NINTHS TO DE LONG & FRENCH, OF NEW YORK, N. Y.

## ASBESTUS-FACED FELT.

SPECIFICATION forming part of Letters Patent No. 387,368, dated August 7, 1888.

Application filed February 21, 1888. Serial No. 264,748. (No specimens.)

*To all whom it may concern:*

Be it known that I, JAMES L. REED, a citizen of the United States, and a resident of Brooklyn, in the county of Kings and State of New York, have invented certain new and useful Improvements in Asbestus-Faced Felt, of which the following is a specification.

My invention relates especially to heat non-conducting coverings for steam-pipes, &c., and has for its object the provision of a covering cheap and simple to make, which will not be affected by the heat of the object wherewith it is used, which shall consist of one fabric or mass that may be cut to accurately fit in place, and which can be very quickly and easily applied.

To attain the desired end, my invention consists, essentially, in an asbestus faced hair-felt, the said asbestus face being worked into the hair and corrugated, ribbed, or scored so as to freely conform to the object to which it is applied, while at the same time the hair is fully protected from contact with the heated surface, all of which will be hereinafter first fully described, and then pointed out in the claims.

In the drawings, Figure 1 is a plan view of a fragment of my improved boiler-covering, and Fig. 2 is a sectional view thereof. Fig. 3 is a sectional view showing it as applied to a pipe.

Like letters of reference, wherever they occur, indicate corresponding parts in all the figures.

35 A is the hair-felt, made in the usual manner. B is the asbestus face felted into the hair and having corrugations or ribs C.

In preparing my improved asbestus-faced felt, I take crude fiber asbestus and reduce it

to a pulp by beating and floating in water until the fibers are separated and become soft and pliable. I then add about one-fourth in bulk of kaolin or ground tale and beat the mass together for three or four hours until it becomes homogeneous. I then add a sufficient quantity of prepared glue to give strength, adhesiveness, and pliability. The hair-felt is placed upon a suitable table and coated with size. The pulp first above described is then spread evenly upon the felt and rolled, worked, or pressed into the same, forming a part thereof. I then, by the application of pressure, form the corrugations or ridges in the asbestus surface, and, after drying, the completed covering is ready to roll up for shipment and for use.

Having now fully described my invention, what I claim as new therein, and desire to secure by Letters Patent, is—

1. As a new article of manufacture, boiler-covering consisting of hair-felt having a face of asbestus pressed therein and forming a part thereof, substantially as shown and described.

2. Hair-felt having a face of asbestus pressed therein, the said asbestus face being corrugated, ribbed, or scored, substantially as shown and described.

3. The combination, with hair-felt, of a fire-proof flexible face worked into the felt, and corrugated, ribbed, or scored, substantially as and for the uses and purpose shown and described.

Signed at New York, in the county of New York and State of New York, this 14th day of February, A. D. 1888.

JAMES L. REED.

Witnesses:

A. M. PIERCE,  
WM. H. WEIGHTMAN.